

May 20, 1930.

F. JARDINE

1,759,509

METHOD OF MAKING PISTONS

Original Filed Sept. 23, 1926



Fig. 1



Fig. 2



Fig. 3



Fig. 4  
INVENTOR  
Frank Jardine  
BY  
Fitch & Watts  
ATTORNEYS

## UNITED STATES PATENT OFFICE

FRANK JARDINE, OF CLEVELAND, OHIO, ASSIGNOR, BY MESNE ASSIGNMENTS, TO THE ALUMINUM COMPANY OF AMERICA, OF PITTSBURGH, PENNSYLVANIA, A CORPORATION OF PENNSYLVANIA

## METHOD OF MAKING PISTONS

Original application filed September 23, 1926, Serial No. 137,194. Divided and this application filed March 19, 1928. Serial No. 262,641.

This invention relates to a method of making pistons and the like. It is particularly adapted to the making of pistons composed of a plurality of different materials which have different co-efficients of expansions and tend to produce great internal stresses in the pistons when cast.

Pistons are frequently made of a plurality of different materials, as for example, aluminum or aluminum alloy pistons, in which are incorporated steel or iron members for restraining or controlling the expansion of the more expandable material. This type of piston is claimed broadly in my co-pending application, Serial No. 47,214, filed July 31, 1925. A common way of forming such pistons is to cast the main parts of the pistons about the control members so that these are at least partly imbedded within the remainder of the pistons. Upon cooling after the casting operation the different materials tend to contract at different rates and thus set up great internal stresses.

It is an object of this invention to provide a method of eliminating from such pistons some of the internal stresses normally set up therein and of relieving substantially all others.

The invention will be better understood from the description of one practical embodiment thereof illustrated in the accompanying drawings, in which:—

Fig. 1 is a side elevation of a finished piston made according to the invention.

Fig. 2 is a longitudinal section thereof taken on the line 2—2 of Fig. 1.

Fig. 3 is a bottom plan view of the piston, and

Fig. 4 is a view similar to Fig. 1, but showing the piston casting before machining.

The piston has a head consisting of a top 1 and a depending annular flange 2 which may be provided with grooves 3 for the usual piston rings (not shown). Also depending from

the head are walls 4 which carry wrist pin

bosses 5 and 6 and are strengthened and stiffened by webs 7 and 8.

Below the piston head is a skirt comprising bearing or thrust faces 9 and 10 which are joined beneath the wrist pin bosses by strap-like connectors 11. Bearing face 9 is shown as integrally joined to walls 4 by webs 12. The bearing faces are tied together and to the boss carrying walls by control members A and B, shown as hollow squares having their ends embedded in ridges 13 on the inside of the bearing faces, and their sides spanning the space between the bearing faces, with the intermediate parts of the sides embedded in the boss carrying walls. The control members are of a material which will cause the diameter of the piston to change only as desired, for instance at the rate of change of the cylinder in which it operates.

The connectors 11 are split at 14 and the splits spanned by arcuate bridges or culverts 15, the splits and culverts allowing for the perimetrical expansion of the skirt.

Bearing face 9 is shown joined to the piston head by a relatively narrow neck or web 16 while bearing face 10 is separated from the head by an air gap 17.

The piston is made as follows:—

The control members A and B are placed in a mold and the balance of the piston cast around them. The different contraction of the various parts of the piston upon cooling, of course, induces severe internal stresses therein. The piston, before machining, is as shown in Fig. 4. Both bearing faces 9 and 10 are joined to the head flange 2 by webs 16 and 18, respectively. These webs are located centrally of the bearing faces and the outer parts of the faces are separated from flange 2 by cored slots 19. These cored slots permit the outer edges of the bearing or thrust faces to adjust themselves independently of the head and so prevent the production of some stresses both in the faces and head.

After casting, one or both bearing faces

may be separated from the head by cutting either or both necks. In the drawings, neck 18 is shown as cut away, separating bearing face 10 from the piston head. This operation 5 relieves some of the stresses within the piston.

After this, the piston is heat treated for a considerable period at a relatively low temperature. A temperature of 300° F. for a 10 period of 50 hours has been found to give satisfactory results. This long heat treatment relieves practically all the remaining stresses. After this heat treatment the piston may be machined without tending to deform itself, 15 thus considerably facilitating its manufacture.

This application is a division of my co-pending application, Serial No. 137,194, filed on or about Sept. 23, 1926, which application 20 contains claims to the article shown in this present application.

While I have described one embodiment of my invention with some particularity, I do not limit myself to the precise details shown, 25 but claim as my invention all variations and modifications thereof coming within the scope of the appended claims.

1. The process of making an insert piston which comprises casting the piston about the 30 inserts, separating at least one bearing face from the piston head, heat treating at about 300° F. for about 50 hours, and then machining the casting.

2. The process of relieving stresses in an 35 insert piston which comprises separating one of the bearing faces of the piston skirt from the head and then maintaining the piston at a temperature of about 300° F. for about 50 hours.

40 3. The process of making an insert piston which comprises casting a piston blank having the bearing faces of the skirt integrally connected with the piston head at their centers and spaced therefrom at their sides by 45 cored slots, separating one bearing face from the piston head, heat-treating at about 300° F. for about 50 hours, and then machining the casting.

4. The process of making an insert piston 50 which comprises casting a piston blank with the bearing faces of the skirt thereof integrally connected to the head at their centers and spaced therefrom at their sides by cored slots, partially machining the blank, heat-treating the blank at about 300° F. for about 55 50 hours, and then finishing the machining of the blank.

5. The process of making an insert piston 60 which comprises casting a blank with bearing faces joined at their centers to the head and spaced therefrom at their sides by cored slots, separating one bearing face from the head to relieve some of the internal stresses, 65 heat treating the blank to relieve substantial-

ly all the remaining stresses, and then machining the same.

6. The process of making an insert piston which comprises casting a blank with bearing faces integrally joined to the head at their centers and spaced therefrom at their sides by cored slots, partly machining the blank, heat treating the same, and then finishing the machining thereof to produce the finished piston.

In testimony whereof I hereunto affix my signature this 14th day of March, 1928.

FRANK JARDINE.

70

75

80

85

90

95

100

105

110

115

120

125

130